

No. 795,216.

Patented July 18, 1905.

## UNITED STATES PATENT OFFICE.

FREDERICK FORSTER, OF NEW YORK, N. Y.

## PROCESS OF CLEANING PRINTING-SURFACES.

SPECIFICATION forming part of Letters Patent No. 795,216, dated July 18, 1905.

Original application filed November 25, 1904, Serial No. 234,307. Divided and this application filed January 13, 1905. Serial No. 240,878.

*To all whom it may concern:*

Be it known that I, FREDERICK FORSTER, of New York, in the county of New York and State of New York, have invented certain new 5 and useful Improvements in Processes of Cleaning Printing-Surfaces; and I hereby declare that the following is a full, clear, and exact description thereof.

This invention is an improved process of 10 cleaning printing-surfaces, particularly lithographic plates, such as aluminium, zinc, German or American printing metal, and other materials used for making printing-surfaces for plate-printing. The process may also be 15 used in cleansing other surfaces and objects, and therefore I do not wish to be restricted specifically to its use for cleaning printing-surfaces.

The invention consists in the novel process 20 of cleaning printing-surfaces, as hereinafter described and claimed.

In my cleansing process I use two cleaning 25 solutions which I shall designate as "solution No. 1" and "solution No. 2." These solutions are compounded as follows:

*Solution No. 1.*—Bichromate of potassium, one part; sulfuric acid, two parts; water, twenty parts.

*Solution No. 2.*—Powdered purified alum, 30 four parts; carbonate of soda, four parts; carbonate of potassium, one part; ten-per-cent. solution gallic acid, ten drops; caustic hydrate of soda, four parts; water, thirty-two parts.

In compounding solution No. 2 I prefer to 35 first mix the alum and water, care being taken to remove or keep out any foreign substances or chemicals. The other ingredients are then added thereto.

As the strength of the chemicals varies some- 40 what, the "actinometer" hydrometer test for solution No. 2 is eighty. The solution of gallic acid is to be used in the proportion stated when each "part" represents an ounce—that is, ten drops of gallic acid to each thirteen 45 ounces of chemicals used, exclusive of water.

For cleaning aluminium, zinc, white-metal,

German printing metal, American printing metal, and all other materials commonly used for lithographic printing purposes in the form of plates I proceed as follows:

First, place the plate in an ordinary asphaltum-lined trough and apply solution No. 1 by pouring same evenly thereover. Let the solution remain on plate for about five minutes, then rub plate with felt or other soft material 55 for the purpose of removing surface dirt. Afterward flush plate with water and finally dry plate.

Second, apply solution No. 2 to the aforesaid plate in the same manner as above, distributing it evenly over plate and rubbing it 6c gently at intervals for six or seven minutes with felt or other soft material which will remove all ink, grease, and other foreign matter. Then flush the plate with water. Again 6: apply solution No. 1 thereto for a minute or two, and afterward give plate a final washing with plain water and put in rack to dry.

The plate thus treated will be thoroughly 7c cleansed and prepared for use for lithographic printing without any other preparation or solution being used and without any rubbing except as stated above.

Having thus described my invention, what I claim as new, and desire to secure by Letters 75 Patent, is—

1. The herein-described process of cleaning printing-surfaces and other objects, consisting in first applying to the surface a solution composed of bichromate of potassium, sulfuric acid and water; then washing the surface; second applying to the surface a solution composed of alum, carbonate of soda, carbonate of potassium, gallic acid, caustic alkali and water, rubbing the surface gently 80 and finally washing and drying the surface.

2. The herein-described process of cleaning printing-surfaces and other objects, consisting in first applying to the surface a solution composed of bichromate of potassium, sulfuric acid and water; then washing and 90 drying the surface; second applying to the

2

surface a solution of alum, carbonate of soda, carbonate of potassium, gallic acid, caustic alkali and water, rubbing it thereon gently and then washing the plate; then again applying the last-named solution to the surface, and finally washing and drying the surface.

In testimony that I claim the foregoing as

my own I affix my signature in presence of two witnesses.

FREDERICK FORSTER.

In presence of  
FRANK C. H. WHITE,  
M. T. BRITTON.